

Oct. 15, 1940.

F. ALBERS ET AL

2,217,829

PHOTOGRAPHIC DEVELOPING PAPER

Filed Feb. 23, 1938

*Fig. 1*

Emulsion sensitized with  
the dyestuffs of  
Example 1



*Fig. 2*

Emulsion sensitized with  
the dyestuffs of  
Example 2



*Fig. 3*

Emulsion sensitized  
with the dyestuffs  
of Example 3



*Fig. 4*

Emulsion sensitized  
with the dyestuffs  
of Example 4



Fritz Albers, Erwin Trabert  
Alfred Sack, Wilhelm Jessien INVENTORS  
Walter Dieterle, Oskar Riester

BY *Albert John*

THEIR ATTORNEYS

Patented Oct. 15, 1940

2,217,829

**UNITED STATES PATENT OFFICE**

2,217,829

## PHOTOGRAPHIC DEVELOPING PAPER

**Fritz Albers, Erwin Trabert, Alfred Sack, and Wilhelm Jessien, Leverkusen-Wiesdorf, Walter Dieterle, Dessau-Ziebigk, and Oskar Riester, Dessau, Germany, assignors, by mesne assignments, to General Aniline & Film Corporation, New York, N. Y., a corporation of Delaware.**

**Application February 23, 1938, Serial No. 192,068  
In Germany March 3, 1937**

5 Claims. (Cl. 95—7)

This invention relates to an improved photographic developing printing paper comprising sensitized silverchloride emulsions and silver-chlorobromide emulsions with or without an addition of silveriodide. Some of these emulsions are cast after washing and some without washing. For adjusting the sensitivity and gradation various ingredients, conditions of ripening and additions are used. Increase of sensitivity in such positive emulsions is limited in consequence of the increasing coarseness of grain and danger of fog which accompany increased ripening. Increasing the sensitivity by the addition of chemical sensitizers has only attained importance in the copying process and is not generally applicable to the more highly sensitive developing emulsions in consequence of danger of fog, diminution of durability and other disadvantages. Optically sensitized emulsions have also been used for making photographic papers for special purposes, for example for copying documents and as material for copying by reflection, as well as for color photography. In consequence of their sensitivity to green-yellow, yellow or red light, such papers cannot be treated in the manner usual for copying purposes in yellow light, and are thus excluded as developing papers in the copying art.

30 It is the object of this invention to increase the general sensitivity of the paper emulsion by adding to the latter an oxothiazolinocarbocyanine which extends the region of spectral sensitivity only in such a manner that it is possible to use  
35 an intense green or yellow darkroom light. It is advantageous to use a dye which produces a steep fall of the spectral curve of sensitivity towards the longer waves of the visible spectrum. These dyestuffs also have the property that they can be easily removed from the photographic layer so  
40 that the picture shows clear whites.

The accompanying self-explanatory drawing illustrates the sensitivity curves of the emulsions of the following examples.

45 The following dyestuffs are examples of those suitable for the invention:

(1)

50



A. II.

|                                                                 |      |
|-----------------------------------------------------------------|------|
| Sensitivity maximum on silverchloride or<br>silverchlorobromide | 4900 |
| Sensitivity extension up to                                     | 5100 |

CC1=CC=C2C=C1C(=O)N2C3=CC=C4C=C3C=C4SC5=CC=C6C=C5C=C6N(C)C

10

A II

Sensitivity maximum on silverchloride or A.U.  
silverchlorobromide 5000 10  
Sensitivity extension up to 5200

(3) *... (3) ...*



18

| Sensitivity maximum on silverchloride or<br>silverchlorobromide | A. U. | 20   |
|-----------------------------------------------------------------|-------|------|
| Sensitivity extension up to                                     | 4950  | 5150 |

Sensitivity extension up to 5150



25

88

A. U.

|                                                                 |      |
|-----------------------------------------------------------------|------|
| Sensitivity maximum on silverchloride or<br>silverchlorobromide | 5050 |
| Sensitivity extension up to                                     | 5050 |

These dyestuffs are made in known manner, for example by the process described in British specification 353,863 accepted July 24, 1931. Photographic papers prepared by this invention may be treated in a darkroom lighted with green or yellow light, for instance light which has passed through Agfa filter No. 113 or No. 112. 35 40

The preparation of gelatine silver bromochloride emulsion is well known to those skilled in the photographic art. To sensitize such emulsions with the dyes herein described, there is prepared a stock solution of the dye by dissolving it in a suitable alcohol, such as methylalcohol. Then into one liter of a developing photographic printing emulsion there is incorporated an amount of the above stock solution (diluted somewhat with water, if desired) containing from approximately 0.03 to about 0.01 gram of the desired dye. This sensitized emulsion may then be coated upon a suitable paper to a suitable thickness and allowed to dry, the details of which are well known to photographic experts. Photographic printing papers so sensitized have properties different from ones heretofore produced by well known methods and hence are of special utility. Furthermore it will be apparent that these dyes may be 45 50 55 60

incorporated in the emulsion by other methods practiced by the art as, for instance, by bathing the paper upon which the emulsion has been coated in a solution of the dye in an appropriate solvent.

5 We claim:

1. Photographic developing printing paper capable of being copied in intense green or yellow dark room light without fogging comprising a 10 gelatin emulsion layer containing a member selected from the group consisting of silver-chloride, silverchlorobromide, silverchloroiodide and silverchlorobromoiodide, and an oxothiazolino trimethinecyanine dye.
- 15 2. Photographic developing printing paper capable of being copied in intense green or yellow dark room light without fogging comprising a gelatin emulsion layer containing a member selected from the group consisting of silver-chloride, silverchlorobromide, silverchloroiodide and silverchlorobromoiodide, and an oxothiazolino 20 trimethinecyanine dye capable of producing a steep fall of the spectral curve of sensitivity towards the longer waves of the visible spectrum.
- 25 3. Photographic developing printing paper capable of being copied in intense green or yellow dark room light without fogging comprising a gelatin emulsion layer containing a member selected from the group consisting of silver-chloride, silverchlorobromide, silverchloroiodide and silverchlorobromoiodide and a dye 30 corresponding with the following formula

35



in which X represents an acid radical.

4. Photographic developing printing paper capable of being copied in intense green or yellow dark room light without fogging comprising a gelatin emulsion layer containing a member selected from the group consisting of silver-chloride, silverchlorobromide, silverchloroiodide and silverchlorobromoiodide and a dye corresponding with the following formula

5



10

in which X represents an acid radical.

5. Photographic developing printing paper capable of being copied in intense green or yellow dark room light without fogging comprising a gelatin emulsion layer containing a member selected from the group consisting of silver-chloride, silverchlorobromide, silverchloroiodide and silverchlorobromoiodide and a dye corresponding with the following formula

20



25

in which X represents an acid radical.

FRITZ ALBERS.  
ERWIN TRABERT.  
ALFRED SACK.  
WILHELM JESSIEN.  
WALTER DIETERLE.  
OSKAR RIESTER.

35